

Dec. 4, 1945.

S. TOUR ET AL

2,390,282

ELECTROLYTIC BARREL PICKLING AND POLISHING

Filed Oct. 19, 1940

Fig:1.



Fig:2.



INVENTORS  
SAM TOUR  
BY ALBERT E. HOWE  
Donald W. Robertson  
ATTORNEY

## UNITED STATES PATENT OFFICE

2,390,282

ELECTROLYTIC BARREL PICKLING AND  
POLISHINGSam Tour and Albert E. Howe, New York, N. Y.,  
assignors, by mesne assignments, to said Tour

Application October 19, 1940, Serial No. 361,930

3 Claims. (Cl. 204—140)

The present invention relates to the electro treatment of metals, and has particular reference to anodic pickling and polishing.

It is the principal object of the invention to provide a practical anodic barrel treatment.

Another object of the invention is to provide a novel combination of electrolyte and metal for anodic barrel treatment.

A further object is to utilize a selected electrolyte and a selected anode to build up a passive 10 anodic layer on the anode.

Still another object of the invention is to utilize a container without previously applied insulating coating for the anodic treatment of metals.

With the above and other objects and advantageous features in view, the invention consists of a novel method and novel combinations of electrolyte and metal anodes more fully disclosed in the detailed description following, and more specifically defined in the claims appended 20 thereto.

The electrochemical treatment of work such as metal articles requires that electrical contact be made with the articles being treated. For quantity treatment of small articles a barrel of non-conductive material, such as hard rubber or Bakelite, is used, and exposed metal contact points or strips are provided in the interior thereof. This type of arrangement may be used for electroplating, electropickling and electropolishing.

In the case of electroplating, metal coats the contacts as well as the articles being plated; whereas in the case of electropolishing and electropickling, metal is removed from the articles being treated as well as from the contacts. Consequently, in the case of electropolishing and electropickling, the contacts are continually being eaten away.

If the work is cathodic in the electrolyte, the passage of the current protects the contact points or strips from electrochemical attack; however, there has heretofore been no protection when the work is anodic, and the passage of current causes an electrochemical attack on the work being treated and on the exposed contact points and strips, which are rapidly eaten away. Anodic pickling by the barrel method has not therefore been heretofore practical.

It has been found that certain combinations of electrolytes and metal anodes eliminate the electrochemical attack and render anodic barrel pickling practicable. The electrolyte first being selected to suit the material of the articles being treated, it is then necessary to select the proper

metal for the contact points or strips or for the entire barrel.

If the metal-electrolyte combination selected utilizes a metal inert to the electrolyte, either with or without passage of the current, no attack on the metal will take place. Thus, platinum may be used in some cases, but it is found that current leaves the entire surface of the platinum whether or not there is work to make contact with, the entire surface area of the immersed platinum becoming effective anode area for the passage of current. If an entire barrel be constructed of platinum, the current loss becomes excessive, and the material cost for ordinary use prohibitive.

With certain combinations of electrolyte and metal, the immersed metal surface becomes passive on the application of the voltages used for anodic pickling or polishing and thus prevents excessive current loss from the exposed immersed surfaces and electrochemical dissolution of the metal used for contact points or strips or for the entire barrel.

Thus, aluminum used as an anode in electrolytes of sulphuric, chromic, oxalic and other acids builds up passivity by formation of an anodic layer of considerable thickness, stability and permanence, the heavy anodic layer being a poor electrical conductor which prevents excess 25 in loss of current from the exposed metal surfaces but which also prevents good electrical contact with the work to be treated.

It is therefore preferred to use combinations of electrolyte and metal where the metal becomes 30 passive and/or forms an anodic film, the passivity being readily broken by physical contact or impact of the metal articles being pickled or polished, or by mounting brushes, wheels, or the like to be contacted.

40 A preferred combination of electrolyte and metal suitable for electropolishing of stainless steel articles is an electrolyte of sulphuric and hydrofluoric acids together, in a barrel constructed of pure copper. If a complete copper 45 construction is adopted, the entire container is a contact point; although a passive coating forms on the copper surface with current flow, the slight impact of the tumbling work is sufficient to break through and establish contact.

50 Copper is easily workable and readily available, and has long life; while not completely passive, commercially pure copper will draw .005 amp./sq. in. if proper conditions are maintained, where stainless steel draws 3.5 amps./sq. in. The 55 passive condition is not as good if copper alloys

are used, or if the electrolyte is too low in sulphuric acid or is allowed to get too hot.

For stainless steel work such as nuts, bolts, screws, etc., the barrel is preferably comparatively small and easy to handle, as the time factor is short and the required current density is high. It is not necessary to rinse the work rapidly, and loading and unloading without rinsing the acid off the barrel is feasible and will prevent introducing water into the electrolyte. Repeated tests have shown no evidence of any "burning" in barrel treatment.

It is preferred to use a potential of 12 to 20 volts, and as high a current density as necessary, as much cathode surface as possible being crowded inside and outside the barrel; heavy gauge woven copper mesh has been found good for this purpose and is placed as close to the work as possible. A lead-lined tank may be used to hold the electrolyte.

Any type of barrel may be used, one preferred form being an adaptation of the oblique plating barrel type, which permits frequent inspection of the work in process.

Another form preferred for the continuous treatment of small parts is of the totally submerged cylindrical barrel type, with a helical internal path. With the work passing through the solution in a thin layer, it is feasible to maintain anodic current densities of 5 to 10 amps./sq. in., and to reduce treatment time to a few minutes or fractions of a minute, with good efficiency and performance.

In the appended drawing I have shown illustrative examples of equipment which can be employed in the practice of my invention. However, it is to be understood that equipment of other types can be employed, for the construction of the apparatus forms no part of the present invention.

Fig. 1 is a schematic sectional view of one form of electrolytic apparatus; and Fig. 2 is a longitudinal sectional view of one particular form of treating barrel which is preferred for the continuous treatment of small parts.

In the apparatus of Fig. 1, a tank 1 provided with a lead lining 2 contains an electrolyte 3. A perforate copper tumbling barrel 4 is obliquely arranged in the tank, as by means of a shaft 5, suitably supported. Heavy gauge woven copper mesh cathode elements 6 and 7 provide cathode surfaces inside and outside the barrel, being placed as close to the work as possible. Frequent inspection of the work may be had by tilting the barrel above the level of the electrolytic bath.

In the form of barrel shown in Fig. 2, the perforate shell 8 is provided with a helical element 9 affording a helical internal path for the parts being treated. The barrel can be totally submerged in the electrolyte, suitable means being provided for introduction and removal of the work. An internal cathode element 10 is mounted on the barrel shaft 11, and of course is insulated from the barrel.

Other examples of electrolyte metal combinations suitable for the electropolishing of metals is the use of an electrolyte of sulphuric and phosphoric acids and a barrel of copper. Copper alloys such as brass or nickel silver, zinc, cadmium or zinc cadmium alloys are also suitable for the described use. Still another example of a suitable anode metal for electrolytes containing sulphuric acid is tantalum.

The basic principles are described above are applicable to electropickling and electropolish-

ing, using racks, baskets, and other types of supports and containers. When containers such as racks and baskets are used the exposed portions act as the contact points. The racks and baskets 5 previously required coating with insulating materials, but the difficulties caused by dissolution of the metal are remedied according to the present invention by making the racks and baskets of a metal which becomes passive in the particular electrolyte used, the passivity being broken or removed, if desired, in any suitable manner.

Although specific combinations of electrolyte and metal have been disclosed which are suitable for anodic treatment, it is obvious that other combinations may be used, according to the work and to the electrolytic treatment and electrolyte most suitable therefor.

We claim:

1. In an anodic electrolytic treatment of the 20 class consisting of electropickling and electro-polishing of metal articles in an electropolishing sulphuric acid-hydrofluoric acid-water electrolyte, the steps of immersing in said electrolyte a barrel electrode of copper, bringing the metal

25 articles into contact with the inside surfaces of the barrel, making the barrel the anode while passing a current through the barrel, articles and electrolyte at a voltage and current density effective in said electrolytic treatment and under 30 conditions which passivate the barrel with respect to the passage of current, and rotating the barrel to produce relative movement and mechanical contact between the articles and barrel to establish electrical contact between the barrel and the articles.

2. In an anodic electrolytic treatment of the 35 class consisting of electropickling and electro-polishing of metal articles in an electropolishing electrolyte of the class consisting of sulphuric acid-hydrofluoric acid-water and sulphuric acid-

40 phosphoric acid-water, the steps of immersing in said electrolyte a barrel electrode of copper, bringing the metal articles into contact with the inside surfaces of the barrel, making the barrel the anode while passing a current through the barrel, articles and electrolyte at a voltage and current density effective in said electrolytic treatment and under conditions which passivate the barrel with respect to the passage of current, and rotating the barrel to produce relative movement and mechanical contact between the articles and barrel to establish electrical contact between the barrel and the articles.

3. In an anodic electrolytic treatment of the 45 class consisting of electropickling and electropolishing of metal articles in an electropolishing sulphuric acid-phosphoric acid-water electrolyte, the steps of immersing in said electrolyte a barrel electrode of a metal of the class consisting

50 of copper, brass, nickel silver, zinc, cadmium, alloys consisting essentially of zinc and cadmium, and tantalum, bringing the metal articles into contact with the inside surfaces of the barrel, making the barrel the anode while passing a current through the barrel, articles and electrolyte at a voltage and current density effective in said electrolytic treatment and under conditions which passivate the barrel with respect to the passage of current, and rotating the barrel to produce relative movement and mechanical contact between the articles and barrel to establish electrical contact between the barrel and the articles.

55 4. In an anodic electrolytic treatment of the class consisting of electropickling and electropolishing of metal articles in an electropolishing sulphuric acid-phosphoric acid-water electrolyte, the steps of immersing in said electrolyte a barrel electrode of a metal of the class consisting 60 of copper, brass, nickel silver, zinc, cadmium, and tantalum, bringing the metal articles into contact with the inside surfaces of the barrel, making the barrel the anode while passing a current through the barrel, articles and electrolyte at a voltage and current density effective in said electrolytic treatment and under conditions which passivate the barrel with respect to the passage of current, and rotating the barrel to produce relative movement and mechanical contact between the articles and barrel to establish electrical contact between the barrel and the articles.